

Feb. 27, 1940.

R. K. HOPKINS

2,191,474

METHOD FOR MANUFACTURING COMPOSITE METAL ARTICLES

Filed Dec. 30, 1937



FIG. 1



FIG. 2



FIG. 3



FIG. 4



FIG. 5



FIG. 6



FIG. 7



FIG. 8

INVENTOR  
ROBERT K. HOPKINS  
BY *Virgil F. Davis*  
ATTORNEY

## UNITED STATES PATENT OFFICE

2,191,474

METHOD FOR MANUFACTURING COM-  
POSITIVE METAL ARTICLESRobert K. Hopkins, New York, N. Y., assignor  
to M. W. Kellogg Co., New York, N. Y., a cor-  
poration of Delaware

Application December 30, 1937, Serial No. 182,461

4 Claims. (Cl. 22—203)

This invention relates in general to composite metal articles and in particular to the manufacture of composite metal articles made up of a metal base of one composition coated with a thickness of metal of a different composition having properties and characteristics superior to those of the metal of the base in the intended service.

This application is a continuation in part of 10 my applications Serial Nos. 64,496, 64,497, and 161,373, filed respectively on February 18, 1936, February 18, 1936, and August 28, 1937.

The present invention contemplates a novel 15 method for obtaining unitary composite articles. In accordance with the method of the present invention a composite article, which may be the final article or the workpiece from which the final article is manufactured, is produced by intimately uniting, throughout the zone of union, the 20 coating metal to the base metal.

In one mode of procedure the metal that is to form the coating is placed in a mold or similar 25 container, with a surface exposed and the molten base metal cast to ultimately cover the exposed surface. The surface of the coating metal exposed to the cast metal is heated to fusion at or approximately at the level of the rising cast metal by an electric current discharge to promote an intermingling of the cast metal and the coating 30 metal into a welded union. The electric discharge may be moved back and forth across the surface of the coating metal and raised with the rising level of the cast metal so that the whole of the surface ultimately exposed to the cast 35 metal is fused with the rising cast metal, alternatively a plurality of closely spaced discharges may be used so that it will only be necessary to raise them. During this operation the electric discharge may be maintained at or slightly above 40 the level of the cast metal. To assure a proper weld between the coating metal and the cast base metal and to protect both from the atmosphere, a blanket of protective flux is maintained over the cast metal as well as over the electric energy 45 discharge. The temperature of the cast metal is preferably so chosen that substantial quantities of the coating metal are not melted by contact therewith so that the depth of the coating metal fused during operation may be more easily controlled.

Alternatively the base metal may be put in the mold in the solidified condition and the coating metal supplied in the molten condition.

The further objects and advantages of the invention will be better appreciated from a con-

sideration of the following description of modes of carrying the invention out in practice taken with the accompanying drawing, in which

Fig. 1 is a schematic view, partly in section, illustrating a manner of carrying out the novel 5 method of the invention;

Figs. 2, 3 and 4 are views, similar to that of Fig. 1, illustrating other modes of carrying out the novel method of the invention;

Figs. 5, 6, 7 and 8 are cross-sectional views of 10 the articles produced in accordance with the invention.

The novel method of this invention may be employed in the manufacture of coated articles of a wide range of compositions. The base metal 15 may be carbon steel, iron, or any of the metals and alloys commonly used in the manufacture of machines, apparatus, vessels, containers, structural members, etc. The coating metal may be of any ferrous or non-ferrous metal or alloy such 20 as chrome steel, manganese steel, chrome-nickel steel, monel metal etc., having corrosion or oxidation, or wear, or other resisting property superior to that of the chosen base metal in the intended service. The articles produced by my novel 25 method, being unitary structures, are admirably suited to withstand the severest service conditions, as for instance, those encountered in the petroleum processing arts where corrosive 30 mediums are handled at temperatures in excess of 1000° F. and under pressures in excess of 1000 lbs. per square inch. The preferred base metal for this class of service will usually be plain carbon steel or carbon-molybdenum steel or low chrome-molybdenum carbon steel; the coating 35 metal for this class of service will usually be chrome steel, chrome nickel steel, monel metal, etc.

The novel method may be employed for manufacturing coated articles that are substantially 40 in their finished form after the coating operation or it may be employed for manufacturing intermediate articles or workpieces such as ingots, slabs, billets, cylinders and the like from which the final articles are produced by working opera- 45 tions such as forging, rolling etc. The articles may be produced in the form of flat members such as slabs, plates, etc., or shaped members such as angles, channels and similar shaped forms, or they may be produced as solid cylinders such as 50 bars or as hollow cylinders such as tubes.

To form a flat surfaced article as, for instance, a thick coated slab from which plate 10, such as shown in Fig. 5, is rolled, the coating metal, as for instance 12—14 chrome steel, in the form of 55

a plate 11 is placed in a rectangular mold 12. Suitable supports (not shown) may be provided in the bottom of the mold to support plate 11. Welding head 14 is moved into position over mold 12. Welding head 14 may be of any preferred construction and arrangement but should be such as to supply current, either A. C. or D. C. or both, of substantially constant amperage and voltage and feed electrode 15 at rates controlled 5 to maintain a discharge of predetermined voltage and amperage. Welding head 14 is provided with electrode feed wheels 16 and includes cables 17 and 18 for passing current to plate 11 and contact device 19 respectively. Contact device 19 10 may be of any preferred construction but is preferably shaped along the lines indicated to direct electrode 15 towards the exposed side of plate 11. Welding head 14 may include a current generator, or generators, or it may be provided with leads to 15 an outside source of current.

Welding head 14 is mounted for vertical as well as longitudinal movement so that electrode 15 may be moved back and forth in a substantially horizontal path across the exposed side of 20 plate 11 and this path raised either continuously or from time to time to maintain it at or slightly above the level of the fused base metal 20. While only one welding head 14 and one electrode 15 have been shown a plurality of these may be employed. If a plurality of electrodes is used their paths may overlap. Whether one or more electrodes will be used will depend on the length of exposed side of plate 11, the purpose being to 25 employ a sufficient number of electrodes 15 to assure that the rising molten metal will always come in contact with fused portions of plate 11 so that an intermingling of the molten metal 20 and the metal molten from plate 11 is guaranteed and a proper weld therebetween is assured.

40 Electrode 15 may be of any shape or character, thus, it may be hollow or solid, round, square etc. Due to its superior penetration an electrode in wire form is at present preferred. Electrode 15 may be of the same or substantially the same 45 composition as the metal of plate 11 or it may be of the same or substantially the same composition as molten metal 20. In view of the small amount of metal deposited from electrode 15 it may not be necessary to compensate for the loss 50 of constituents thereof in the electric discharge, however, it is contemplated that such compensation may be made when necessary. While, in general, electrode 15 will be of the composition as stated, it need not always be so as it may be 55 made of substantially non-consumable materials such as carbon or tungsten. The use of this type of electrode will be governed by the effects of the carbon or tungsten contaminations on the molten metal.

60 After welding head or heads 14 are moved into position electrode 15 is fed until it almost touches plate 11. An arc starter, such as a ball of steel wool, a nail or the like, is interposed between the end of the electrode and the surface of plate 11. A deep blanket of flux 13 is then placed 65 in the bottom of the mold to cover the whole of it to a depth of several inches or more.

70 Flux 13 should be such that it will not liberate deleterious gas, either as to quantity or kind, when molten or when in contact with molten metal or under the influence of the heat generated by an electrical energy discharge. Flux 13, furthermore, should be such that it will not add substantial quantities of undesirable ingredients 75 to or remove desirable ingredients from the mol-

ten metal but will flux out impurities. A wide variety of fluxes may be used satisfactorily. Silicates, in general, either simple silicates and mixtures thereof, or complex silicates and mixtures thereof, are satisfactory. Aluminates, titanates and similar compounds are likewise satisfactory and may also be used in mixture with silicates. The flux may also include thinning compounds such as feldspar and the like. The flux need not be composed of reacted materials 10 but may be made up of their dried or calcined unreacted components. Thus, in the case of calcium silicates the flux may be made up of CaO and SiO<sub>2</sub>, in the case of manganese silicates, it may be made up of MnO and SiO<sub>2</sub>. At present, 15 silicates of the alkaline earth metals, and manganese, aluminum, and iron are preferred as fluxes. Flux blanket 13 may be placed in the mold in the solidified condition and in broken up form, also it may be placed in mold 12 in the molten 20 condition. After the flux blanket 13 is laid the electrical circuit is closed. The initial surge of current will destroy the arc starter and provide a path for the passage of current between the end of the electrode and the surface of plate 11. 25 The electric current discharge will melt metal of the electrode and metal of the surface of plate 11; the current discharge will also melt some of the flux, when the flux is in the solidified condition or raise its temperature when it is molten. The 30 welding head, or heads 14 will be moved back and forth so that a substantially continuous horizontal band of metal of plate 11 will at all times be in the molten condition. A continuous band 35 of molten metal may also be obtained without oscillation of the electrodes by employing a sufficient number of closely spaced, and preferably small, electrodes.

Molten metal 20 is then poured into mold 12. The molten metal is preferably at a temperature 40 proper for pouring and is not superheated so that it will have a minimum tendency to fuse the solid portions of plate 11. In this manner, the penetration into plate 11 is controlled and maintained throughout the height of plate 11. The pouring 45 of molten metal 20 and the raising of welding head 14 are so synchronized or controlled that the discharge of electric current will always be at the proper elevation with respect to the level of the molten metal 20 so that the heat of the 50 discharge will not only provide molten metal from plate 11 to commingle and become a part of molten metal 20 but will raise the temperature of the molten metal 20 in contact with plate 11 high enough to assure this result. 55

Thus the electric discharge may be on at or slightly above the level of molten metal 20 and make take place between electrode 15 and metal 11, or between electrode 15 and metal 11 as well as molten metal 20, or between electrode 15 and 60 molten metal 20. Various arrangements may be employed for maintaining the discharge at the predetermined elevation relative to the level of the molten metal 20. At present, I prefer to employ a non-consumable water cooled electrode 65 and discharge current through a gap between it and molten metal 20, the electrode being retracted by automatic means to maintain the voltage of the discharge constant. The rate of retraction of this electrode will be exactly equal to the 70 rate of rise of molten metal 20 and by raising head 14, as through electrically actuated means, in accordance with the retraction the predetermined elevation will be maintained.

To further assure the maintenance of a uni- 75

form penetration throughout the height of plate 11 passageways 23 are provided in the walls of mold 12 for the passage therethrough of a heat exchange medium such as water. These passageways are preferably so connected that the heat exchange medium can be circulated through any of the sides or bottom of mold 12 independently. Thus, the side of mold 12 against which plate 11 rests may be cooled by the circulation of heat exchange medium to prevent a melting of plate 11 to a depth beyond that contemplated by the intensity of the current discharge and the other sides and bottom of mold 12 may be cooled when it is desired to accelerate the cooling and solidification of the cast metal.

The molten metal 20 may be poured through flux blanket 13 or it may be poured from beneath flux blanket 13. If molten metal 20 is poured from beneath, it may be poured from a ladle 21 through the conduit 22 indicated in dotted lines on Fig. 1. In this event, heat exchange medium is not circulated through the bottom and sides of mold 12 other than that side against which plate 11 rests. Molten metal 20 may also be poured from ladle 21 through conduit 22 and flux blanket 13. In this case, all of the sides and bottom of mold 12 may if desired, be cooled. The advantage of the latter mode of operation is that the molten metal 20 is solidified progressively as the level rises in mold 12 and if the operation is properly controlled a minimum of molten metal will be present in mold 12 at the end of the operation. This means that a minimum of shrinkage cavities will be present in the cast metal 20. To assure high grade metal up to the top of plate 11 mold 12 may, if desired, be provided with a shrink head or similar device (not shown).

After the molten metal has solidified the resultant article which corresponds to a coated slab is removed from mold 12 either for direct use or for working into the final desired article. The slab thus formed will include as the major portion of its thickness base metal 20 to which is intimately and thoroughly united throughout coating metal 11. The union between the coating metal and the base metal is so thorough and complete that the slab is to all intents and purposes, a unitary structure.

The slab thus formed will usually be rolled or otherwise worked into plates, sheets or the like. The working operation will not only produce an article of desired shape and size but will also convert the cast metal into work refined metal. For economical reasons the slab will, in general be made many times thicker, as for instance, from 10 to 20 times or more, than the finally desired article so that there will in the working be a substantial reduction in thickness and a proportionate reduction in the cost of the operation when figured on unit of area of the final article.

As shown, particularly in Fig. 2, the operation may be so carried on to produce an ingot from which two plates 10 may be rolled. In this case, a pair of plates 11 is assembled as by welding and a space 24 provided between them for the circulation of water or other heat exchange medium. Welding heads 14 and electrodes 15 are provided on each of the exposed sides of assembled plates 11 so that metal of both of the exposed surfaces may be simultaneously melted to commingle with the rising molten metal 20. As disclosed in connection with Fig. 1, the molten metal may be bottom poured or top poured. If

bottom pouring is employed the heat exchange medium is not circulated through the sides and bottom of the passageways in mold 12. If top pouring is employed a heat exchange medium may be circulated through all of the passageways to accelerate the cooling and solidification of the cast metal. In either case heat exchange medium is circulated through space 24 between the plates 11. When the operation is completed the ingot is removed from the mold. The ingot may be worked directly and plates 11 separated after working, or the ingot may be separated into slabs and the slabs may be separately worked to form plates 10. When the ingot is worked directly it will be found preferable to coat at least one of the opposed surfaces with any of the usual compounds to prevent welding of plates 11 during the working operation.

The arrangements of Figs. 3 and 4 are intended for the production of unitary composite bodies, which may be final products or workpieces from which final products may be manufactured, having a core of metal of one composition surrounded or enveloped by metal of another composition. The molds 12 and welding heads 14 of Figs. 3 and 4 are of the same character as those of Figs. 1 and 2. However, molds 12 will be of a cross section to correspond with that of the composite body to be produced, thus, the cross-section of these molds may be rectangular, circular or polygonal. In the apparatus of Figs. 3 and 4 welding heads 14 and molds 12 are so arranged relative to each other that electrode 15 will move through a helix like path so that they can completely cover the exposed surface of the coating metal. When core 25 (Fig. 3) is cylindrical the electrode path will be a helix, when annulus 26 (Fig. 4) is circular the electrode paths will also be a helix. As in the case of the arrangements of Figs. 1 and 2 a sufficiently large number of small electrodes may be employed to give a substantially continuous band of fused metal and the electrodes merely raised to maintain the predetermined elevation relative to the molten metal 20.

The arrangement of Fig. 3 is specifically intended to produce a composite body having a core 25 to which is united an envelope of cast metal 20. Such a body will generally serve as a workpiece from which the internally coated seamless tube 27 of Fig. 7 may be manufactured. In the usual case the composite body is opened through its center as by passing through a Mannesmann mill, or by trepanning, etc., to form a thick walled tube and the final seamless tube 55 made by rolling the thick walled tube to the desired dimensions. Tube 27 may also be drawn or cold rolled as desired.

The arrangement of Fig. 4 is specifically intended to produce a composite body having an envelope 26 to which is united a core of cast metal 20. Such a body will generally serve as a workpiece from which externally coated seamless tube 28 of Fig. 6 may be manufactured. Generally the composite body is first opened through its center as by passing it through a Mannesmann mill, or by trepanning, etc., to form a thick walled tube which is rolled into the final tube 28 of desired dimensions. Tube 28 may also be drawn or cold rolled if desired.

When carrying out the novel method with the arrangements of Figs. 3 and 4 the cast metal 20 may be top poured or bottom poured. With top pouring penetration can be better controlled and shrinkage defects minimized by circulating a cool-

ing medium through tubes 23 in the walls and bottom of molds 14. In Fig. 3 core 25 may have a central passageway through which a cooling medium may be circulated to facilitate the control of penetration.

Workpieces from which internally and externally coated seamless tube 29 of Fig. 8 are manufactured may be made by combining the procedure illustrated in Figs. 3 and 4. In making such workpieces a core is centered in the mold as in Fig. 3 and an annulus placed against the mold sides as in Fig. 4; the cast metal is poured in the space between the annulus and core. To unite the cast metal to the core an electrode or electrodes are rotated around the core beneath a blanket of flux and the current discharged to fuse a depth of the core so as to obtain a union between the cast metal and the core metal. An electrode or electrodes are also rotated proximate the inner wall of the annulus beneath a blanket of flux and the current discharged to fuse a depth of the annulus so as to obtain a union between the cast metal and the metal of the annulus. Again a plurality of small closely spaced electrodes may be employed. The seamless tube 29 is made by working as explained in connection with tubes 27 and 28. Tube 29 may have an inner coating 30 of one composition and an outer coating 31 of a different composition, or if desired, coatings 30 and 31 may be of the same composition.

In the above description the cast metal has been chosen as the base metal for in the coating of steel base metal with protective alloys such as chrome steels and chrome nickel steels usually better results are obtained. However, the invention is not limited to this for the coating metal may be cast and the base metal placed in the molds in the solidified condition. Generally, the metal or higher melting point will be placed in the mold in the solidified condition and the metal of lower melting point cast in the mold. By following this rule troubles due to excessive fusion of the solid metal will be avoided and penetration into the solid metal more accurately controlled.

I claim:

1. The method of uniting metals which comprises, providing a mold space defined at least in part by a non-horizontal surface of a solid metal body, pouring molten metal into said mold space beneath a blanket of protective flux therein to progressively cover said non-horizontal surface, the molten metal being supplied from a molten metal source external to said mold space, and uniting the metals by fusing a depth of the solid metal defining said non-horizontal surface as

the molten metal is poured to intermingle the metals, the fusion of the solid metal being effected by the discharge of electric current through a gap beneath the surface of the blanket of flux.

2. The method of manufacturing metal articles which comprises, providing a mold space defined at least in part by a non-horizontal surface of a solid metal body, pouring molten metal into said mold space beneath a blanket of protective flux therein to progressively cover said non-horizontal surface, the molten metal being supplied from a molten metal source external to said mold space, and uniting the metals by fusing a depth of the solid metal defining said non-horizontal surface at substantially the molten metal level as said molten metal rises to cover said non-horizontal surface, the fusion of the solid metal being effected by the discharge of electric current through a gap beneath the surface of the flux blanket.

3. The method of manufacturing metal articles which comprises, providing a mold space defined at least in part by a non-horizontal surface of a solid metal body, pouring molten metal into said mold space beneath a blanket of protective flux therein to progressively cover said non-horizontal surface, the molten metal being supplied from a molten metal source external to said mold space, fusing a depth of the solid metal in the zone of the meeting line of said non-horizontal surface and the molten metal surface as the molten metal rises in the mold space, the fusion of the solid metal being effected by the discharge of electric current through a gap beneath the surface of a blanket of flux, said gap being positioned sufficiently adjacent the solid metal to fuse the solid metal directly by the heat generated at the gap.

4. The method of manufacturing metal articles which comprises, providing a mold space defined at least in part by a non-horizontal surface of a solid metal body, pouring molten metal into said mold space beneath a blanket of protective flux therein to progressively cover said non-horizontal surface, the molten metal being supplied from a molten metal source external to said mold space, discharging electric current beneath the surface of the blanket of flux through a gap between the end of a fusible metal electrode and the metal in the zone of the meeting line of said non-horizontal surface and the molten metal surface to fuse a depth of the solid metal defining said non-horizontal surface directly by the heat of the discharge, whereby the metals are intermingled, and controlling the dissipation of heat from the metals to fuse a substantially constant depth of the solid metal.

ROBERT K. HOPKINS.